

March 4, 1952

A. M. GUNDELFINGER

2,587,841

PHOTOGRAPHIC TONING AND RESENSITIZING PROCESS

Filed Oct. 6, 1947



Fig. 1. ↓ FIRST TONING STEP



Fig. 2. ↓ SECOND TONING STEP



Fig. 3. ↓ RESENSITIZING STEP



Fig. 4.

Alan M. Gundelfinger

BY Silvander and Matherly

ATTORNEYS

## UNITED STATES PATENT OFFICE

2,587,841

## PHOTOGRAPHIC TONING AND RESENSITIZING PROCESS

Alan M. Gundelfinger, Los Angeles, Calif., assignor to Cinecolor Corporation, Burbank, Calif., a corporation of California

Application October 6, 1947, Serial No. 778,269

5 Claims. (Cl. 95—88)

1

My invention relates generally to the art of photography and particularly to processes of producing colored photographs in which two or more images are produced in the same emulsion.

In various color processes it is customary to first print one color component image in a photographic emulsion layer and then after developing said image, to print a second image to the same emulsion, it usually being advisable to regenerate the emulsion prior to the second printing operation. In some instances the first image is colored by toning or other convenient process prior to the second printing operation, and in some cases it is converted to a form which will be more stable during subsequent operations.

The first image printed to the photographic emulsion is usually of variable density, that is to say, some portions of the image are of greater depth than others. In printing through such a variable depth image to produce a second image, more light is of course needed in those portions of the film where the first image is of greater density. However, I have found that often in producing a satisfactory second image through the denser portions of the first image, overexposure is obtained in those portions of the film where the first image is relatively thin or is not present at all.

An object of my invention is therefore to provide a method of selectively increasing the sensitivity of a photographic emulsion in proportion to the density of a variable density image therein.

Another object of my invention is to provide a method of producing a first image in a color process, which image when the emulsion is regenerated, will cause the resultant sensitivity of the film to be substantially proportional to the depth or density of said first image.

Stated another way, it is an object of my invention to provide a method of sequentially producing two or more photographic images in a single emulsion, the first image being used to modify the sensitivity of the film so that it is substantially proportional to the masking effect of the first image.

A further object of my invention is to provide a multiple step toning process for accomplishing the foregoing objects.

My invention finds one of its most important applications in color processes involving the toning and/or dye toning of one or more images in the same emulsion and I have found it particularly valuable in processes wherein the first image produced in the emulsion is iron-toned to produce a Prussian blue image.

2

In general, the preferred form of my invention as applied to a process employing iron-toning of the first image and dye toning of the second image, contemplates producing a first latent image principally in the outer strata of a photographic emulsion, developing said image, toning the image Prussian blue in a plurality of steps as hereinafter set forth in detail, converting said Prussian blue image to a ferric hydroxide or other inert image, reconverting the silver ferrocyanide formed by the reaction of the toning bath and the silver image to silver bromide, printing the second image to the surface of said emulsion, developing said second image, toning or dye toning the second image and finally restoring the proper color to said first image.

As those skilled in the art are well aware, light-sensitive silver halide crystals may be formed from the silver ferrocyanide produced by toning, as mentioned in the preceding paragraph, with either an alkaline reagent such as that described more particularly hereinafter, or an acidic reagent such as those taught in U. S. Patent No. 1,538,816 to Ives.

It is known that the sensitivity of a photographic emulsion is sometimes increased when the light-sensitive silver halide crystals therein are formed in the presence of highly dispersed insoluble particles in the emulsion. It is thought that this increased sensitivity is due to the presence of insoluble particles, adsorbed on the surface of the silver halide crystals. These adsorbed particles serve a twofold purpose, namely to set up crystal lattice strains necessary for latent image formation and to act as developing nuclei. With this fact in mind I convert the first silver image produced in the emulsion to an insoluble silver salt in the presence of other insoluble and relatively smaller particles, the dispersion of which varies directly with the density or depth of the image. The variation in dispersion of these particles can of course be accomplished uniformly by variation of the treating bath during conversion, but from a practical standpoint it is advisable to produce this differential sensitivity in steps or stages. In other words, by converting the first image, in the emulsion, in such a manner that the outer strata thereof are composed of particles such as grains or granules which are relatively less dispersed, and the inner or deeper strata of the image are composed of relatively highly dispersed particles (approaching a molecular dispersion), we produce a light sensitive layer,

the inner strata of which will have a higher de-

gree of sensitivity than those strata near the surface of the image.

Considering now in detail one preferred form of my invention, the photographic emulsion is exposed to an appropriate color separation negative to produce a latent color-component image in the printed film, which image is then developed, washed, hardened and partially iron-toned by any convenient method. A suitable solution for this partial toning operation is as follows:

*First toning solution*

|                                 |       |          |
|---------------------------------|-------|----------|
| Potassium ferricyanide          | gms.  | 10 to 15 |
| Ferric ammonium sulphate        | gms.  | 14       |
| Potassium alum (or chrome alum) | gms.  | 14       |
| Potassium oxalate               | gms.  | 19       |
| pH (provided by sulphuric acid) |       | 1.5      |
| Water                           | liter | 1        |

Treatment of the silver image in the above solution converts the outer part or stratum of the image to a mixture of ferric ferrocyanide (Prussian blue) and silver ferrocyanide. The film is removed from this bath prior to the conversion of all of the silver, and at approximately the time when the portions near the surface of the image have been completely toned but before the deeper portions of the image have been completely toned.

The film is then treated with a second toning solution in which the formation of the ferric-ferrocyanide proceeds at a relatively slower rate. From the second treatment with the second solution a higher degree of dispersion of the precipitated ferric ferrocyanide is obtained. This second solution may take one of several forms, all of which, however, act on the same general principle. Four illustrative toning solutions are here listed and the operations and actions of each will be considered separately.

*Second toning solution*

|                                       | A     | B     | C     | D     |
|---------------------------------------|-------|-------|-------|-------|
| Potassium Ferricyanide, gms.          | 10-15 | 10-15 | 10-15 | 10-15 |
| Ferric Ammonium Sulphate, gms.        | 7     | 14    | 14    | 14    |
| Potassium Alum (or Chrome Alum), gms. | 14    | 14    | 7     | 14    |
| Potassium Oxalate, gms.               | 19    | 36    | 19    | 19    |
| pH (provided by sulphuric acid)       | 1.5   | 1.5   | 1.5   | 2     |
| Water, liters.                        | 1     | 1     | 1     | 1     |

As with the first toning solution, the potassium ferricyanide oxidizes the metallic silver to produce silver ferrocyanide and potassium ferrocyanide. The oxalate ions combine with ferric ions to form ferric oxalate complex ions, and the ferric ions which do not enter into the ferric oxalate complex combine with ferrocyanide ions to form ferric-ferrocyanide (Prussian blue). It is the rate of formation of this ferric-ferrocyanide which must be controlled and I have found that the best method of controlling the same is to control the number of ferric ions available at any instant for reaction with the ferrocyanide ions.

Considering first the bath defined in column A above, it will be noted that the amount of ferric ammonium sulphate is relatively low as compared to the first toning solution, thereby giving a relatively low total concentration of ferric ions in solution. With a low concentration of ferric ions the reaction forming ferric-ferrocyanide proceeds relatively slowly and the resulting image is highly dispersed. This is perhaps the most obvious method of slowing down the rate of formation of the ferric-ferrocyanide.

In the formula given in column B it will be noted that the amount of ferric ammonium sul-

phate is the same as in the first toning solution. However, it will also be noted that the amount of potassium oxalate has been increased which means that there are a greater number of oxalate ions available to combine with ferric ions to form ferric oxalate complex ions. This results in a net decrease of ferric ions available at any instant for reaction with ferrocyanide ions which causes the process to proceed more slowly and hence a higher degree of dispersion in the resulting image is obtained.

In the example given in column C, the speed of the reaction is controlled by decreasing the amount of alum (potassium or chromium alum-nium sulphate) with the result that less of the oxalate ions are used in forming aluminum or chromium oxalate complex and consequently there are more oxalate ions to combine with the ferric ions to form ferric oxalate complex. This results in a net decrease of ferric ions available at any instant for reaction with the ferrocyanide ions which causes the process to proceed more slowly and hence a higher degree of dispersion in the resulting image is obtained.

Referring now to the formula given in column D it will be noted that the pH of the solution is higher, i. e., the hydrogen ion content is lower than in the first toning solution. With this lower concentration of hydrogen ions, fewer oxalate ions combine with the hydrogen ions to form oxalic acid, thus leaving a greater number of oxalate ions to combine with ferric ions to form the ferric oxalate complex. Consequently, there are fewer ferric ions present at any instant in the solution for the formation of ferric ferrocyanide and the reaction proceeds relatively slowly, resulting in a highly dispersed image.

The invention will be better understood by reference to the accompanying drawings showing one mode of carrying out the process of invention in which two sequential toning steps are employed.

Figure I is a side elevation of a photographic emulsion situated upon a conventional film support and having a developed silver image present therein.

Figure II is a similar view illustrating the emulsion subsequent to the first toning step in which an upper stratum of the developed silver image is toned to produce relatively coarse ferric ferrocyanide particles and silver ferrocyanide particles.

Figure III is a similar view showing the emulsion subsequent to the second toning step in which the stratum of the developed silver image disposed below the stratum toned by the first toning step has been converted to relatively fine ferric ferrocyanide particles and silver ferrocyanide particles.

Figure IV is a similar view illustrating the emulsion subsequent to resensitization after the second toning step. It will be observed that the resensitized emulsion embraces an upper stratum containing relatively coarse ferric hydroxide and silver halide particles and a lower stratum embracing relatively fine ferric hydroxide particles and silver halide particles.

It will be understood of course that the foregoing examples are merely illustrative of various ways of controlling the speed of formation of the Prussian blue image and that other variations and combinations of toning solutions can be used. Likewise, it will be understood that if other metallic tones such, for example, as nickel, copper, cobalt, uranium, etc., are desired, that appropri-

ate formulas will be used in which the solution for the first stage of the toning operation may be substantially conventional and the subsequent solution or solutions will be adapted to convert the balance of the toned images more slowly, resulting in the image being more highly dispersed in its deeper strata. Since there are a large number of known metallic toning solutions it is believed unnecessary to give further examples.

It will also be understood of course that the conversion of the silver image may be accomplished in three or more steps or stages if desired, by appropriately varying the solutions and time of treatment in each. However, in most cases a two-stage treatment is sufficient.

Since the silver ferrocyanide formed by the reaction of the blue toning solution on the silver image is insensitive to light and is spontaneously redevelopable in developing solutions while silver bromide is light sensitive and relatively much less susceptible to spontaneous development, it is necessary to convert the silver ferrocyanide to silver bromide. This may be accomplished in one of two ways; by adding a soluble bromide to the blue toning solutions, or by treating the film subsequent to the blue toning step with a solution of soluble bromide such as for example, a 2½% solution of potassium bromide. The latter method is preferred because as can be seen from the chemical reactions involved in the blue toning step the contrast of the blue toned image may be maintained at a lower value consistent with good color reproduction. The solution used to convert the silver ferrocyanide may be alkaline in character as more particularly described herein-after, or an acidic medium such as those taught in U. S. Patent No. 1,538,816 to Ives. As previously stated, the silver bromide which is formed in the deeper strata of the image is more sensitive than the silver bromide formed in the outer strata of the image since that in the deeper strata is formed in the presence of more highly dispersed insoluble particles.

Since the ferric ferrocyanide is subsequently affected by the developing solution for the second image in such a manner that it is converted partially to ferric hydroxide and partially to ferrous hydroxide, depending upon the relative quantities of reducing agent or agents and hydroxyl ions of the developer, and therefore results in a non-uniform restoration of the original amount of ferric ferrocyanide in later steps in the process, it is desirable to convert the ferric ferrocyanide completely to ferric hydroxide prior to the second development stage because of the extremely small solubility product of the latter which makes it substantially non-reactive with reducing agents. One method of accomplishing this result is to treat the film with an alkaline solution, such as, for example, a 2.5% solution of sodium carbonate which converts the Prussian blue to ferric hydroxide.

If desired, the conversion of the ferric ferrocyanide to ferric hydroxide and the re-sensitizing of the film may be carried on in one step by using a solution composed substantially as follows:

|                         |       |    |
|-------------------------|-------|----|
| Sodium carbonate -----  | grams | 25 |
| Potassium bromide ----- | do    | 25 |
| Water -----             | liter | 1  |

The degrees of dispersion of the ferric hydroxide image will be substantially the same as the degrees of dispersion of the previously produced ferric ferrocyanide image and consequent-

ly the sensitivity of the film will be proportional to the depth of the hydroxide image. After either of the foregoing treatments the film may be washed and dried and is then ready for the second printing operation.

After the second printing operation the latent image produced thereby is developed and colored by any convenient process such as toning or dye toning, and the ferric hydroxide of the original image may then be reconverted to Prussian blue, as described in United States Patent No. 2,218,001.

When in the claims, I use the term "insoluble" in referring to a salt or other substance, it will be understood that I mean relatively insoluble in the particular solutions used in the process, and not necessarily insoluble in all known solutions.

While I have shown and described a preferred form of my invention, it will be apparent that modifications may be made therein without departing from the broad features as herein defined. Consequently, I do not wish to be restricted to the particular theories or processes herein described, except as limited by my claims.

25 I claim:

1. In a process in which a plurality of developed silver images are sequentially produced in a silver halide photographic emulsion by printing a first latent image in said emulsion, developing and toning said first image to ferric ferrocyanide, converting the toned first image to a ferric hydroxide image, resensitizing the emulsion by converting the silver salts present therein to a silver halide, printing a second latent image in the resensitized emulsion with light for which said ferric hydroxide image has high absorption; the method of improving the quality of said second image by imparting to said resensitized emulsion a sensitivity substantially directly proportional to the masking effect of said ferric hydroxide, which consists essentially of conducting said toning with a plurality of toning solutions in successive toning steps including treating said developed first image, in a first toning step, with a first toning solution containing ferric ions, ferricyanide ions, and a complexing reagent for said ferric ions which suppresses the availability thereof for reaction to form ferric ferrocyanide, said first toning step being so controlled as to convert a portion of said developed first image to coarse ferric ferrocyanide particles confined to a surface layer of said emulsion, and subsequently treating said developed first image in a further toning step with a second toning solution containing ferric ions, ferricyanide ions, and a complexing agent for said ferric ions, the proportion of complexing reagent to ferric ions being greater in said second toning solution than in said first toning solution at the conclusion of said first toning step to make a smaller number of ferric ions available to the ferric ferrocyanide precipitate forming reaction and effect precipitation of ferric ferrocyanide at a slower rate than in said first toning step, said further toning step being so controlled as to convert an additional portion of said image to particles of ferric ferrocyanide of smaller size than those resulting from said first toning step and confined to a layer in said emulsion disposed below said surface layer, the relationship between the particle size of ferric ferrocyanide produced in said toning steps being such as to substantially completely compensate for the masking effect of the ferric hydroxide image.
2. The process of claim 1 in which the complexing reagent comprises oxalate ions.

3. The process of claim 1 in which the emulsion is resensitized by treatment with bromide ions to convert the silver ferrocyanide to silver bromide.

4. The process of claim 1 in which the emulsion is resensitized by treatment with an aqueous solution of potassium bromide.

5. The process of claim 1 in which the emulsion is resensitized with an alkaline aqueous solution containing bromide ions to convert the silver ferrocyanide to silver bromide and the ferric ferrocyanide to ferric hydroxide.

ALAN M. GUNDELFINGER.

REFERENCES CITED

The following references are of record in the file of this patent:

UNITED STATES PATENTS

| Number    | Name | Date           | 20 |
|-----------|------|----------------|----|
| 1,278,668 | Ives | Sept. 10, 1918 |    |

| Number    | Name                | Date           |
|-----------|---------------------|----------------|
| 1,279,276 | Crabtree            | Sept. 17, 1918 |
| 1,538,816 | Ives                | May 19, 1925   |
| 1,623,123 | Loge                | Apr. 5, 1927   |
| 1,695,284 | Ives                | Dec. 18, 1928  |
| 1,930,141 | Capstaff            | Oct. 10, 1933  |
| 1,934,779 | Townsend            | Nov. 14, 1933  |
| 1,945,772 | Dossonville         | Feb. 6, 1934   |
| 2,218,001 | Gundelfinger et al. | Oct. 15, 1940  |
| 2,226,639 | Schinzel            | Dec. 31, 1940  |
| 2,272,556 | Gundelfinger        | Feb. 10, 1942  |
| 2,341,079 | Butement            | Feb. 8, 1944   |
| 2,396,726 | Tremble             | Mar. 19, 1946  |
| 2,415,626 | Coote               | Feb. 11, 1947  |
| 2,444,567 | Huslk               | July 6, 1948   |

OTHER REFERENCES

Mees: The Theory of Photographic Process, pages 576 and 577.